

April 28, 1925.

E. E. HEDGES

1,535,468

## PROCESS OF EXTRACTING SULPHUR FROM ITS ORES

Filed Nov. 29, 1922



## UNITED STATES PATENT OFFICE.

EDWARD E. HEDGES, OF NEW YORK, N. Y., ASSIGNOR TO THE HEDGES NEW EDUCATION PROCESS CORPORATION, OF NEWARK, NEW JERSEY.

## PROCESS OF EXTRACTING SULPHUR FROM ITS ORES.

Application filed November 29, 1922. Serial No. 604,042.

*To all whom it may concern:*

Be it known that I, EDWARD E. HEDGES, a citizen of the United States, residing at New York, in the county of New York and State 5 of New York, have invented certain new and useful Improvements in Processes of Extracting Sulphur from Its Ores; and I do hereby declare the following to be a full, clear, and exact description of the invention, 10 such as will enable others skilled in the art to which it appertains to make and use the same, reference being had to the accompanying drawings, and to the letters and figures of reference marked thereon, which form a 15 part of this specification.

This invention relates to the extraction of sulphur from its ores and has for an object to confine the sulphur ore in a retort closed against the introduction of air, which 20 said retort is heated to a sufficient temperature to liberate the sulphur in vapor form, passing the vapor to a condenser to condense the sulphur and discharging the spent residuum.

25 A further object of the invention is to introduce sulphur ore preferably in finely divided condition into a rotating retort which is maintained at a sufficient temperature to drive off the sulphur in vapor form 30 which is conducted to a condenser and there condensed, and providing means for discharging the spent ores from the retort without the introduction of air either at the charging or discharging.

35 With these and other objects in view the invention comprises certain novel steps in the process, as will be hereinafter more fully described and claimed.

As an apparatus for carrying out the present invention but without limiting the same 40 to said apparatus, the drawings show at:

Figure 1 a longitudinally sectional view taken through a retort and condenser;

45 Figure 2 a transverse sectional view through the retort showing the means for introducing the superheated steam, maintaining the retort in heated condition and discharging the spent residuum.

Like characters of reference indicate corresponding parts throughout the several views.

The present process is carried out in a 50 closed retort which is heated to a sufficient temperature to drive off the volatilizable constituents. In the drawing such a retort

is shown as a cylinder 10 having ribs 11 serving to support the retort upon rollers 12, whereby the said retort may be conveniently rotated in any approved manner and from any approved source, as conventionally indicated by a pinion 13 engaging a beveled gear 14 rigidly secured to the retort.

Preferably the retort will be provided with ribs 15 in its interior by the use of which when the retort is rotated the contained material will be cascaded. The showing of the retort in the drawing as setting substantially upon a horizontal axis is no limitation and the retort may be inclined as may be found necessary to advance the material therethrough, or other means ordinarily known in the art may be employed for the purpose. At the inlet end the retort is provided with a central opening 16 into which is introduced a cylindrical feed conduit 17 having some means therein for advancing the material therethrough from the hopper 18, such means being shown conventionally as the worm 19 driven by the sprocket chain 20. Preferably this conduit 70 17 will be surrounded and insulated by some refractory material, indicated conventionally at 20'.

This feed conduit 17 extends through the condenser 21. The condenser 21 may assume any form which convenience may make desirable or experience may dictate. It is here shown as a chamber inclined somewhat to the axis of the retort having a flue 22 so that the non-condensable gases passing from the retort through the opening 16 into the condenser may escape through this flue. Means for discharging the material 90 from the condenser will naturally be provided and is here shown as a hinged cover 95 23 and means for cutting off the lower part of the condenser chamber for the purpose of discharging the condensates without interrupting the action. The retort is provided with means for automatically and continuously discharging the spent material forming meanwhile a seal against the escape of gases, such discharge being in the form of a volute passage 25 having one end opening at 26 into the interior of the retort 100 and its opposite end opening at 27 into the discharge bell 28.

Extended axially through this end of the retort is a steam pipe 29 preferably branched within the retort, as indicated at 110

30 to form a means for introducing and distributing superheated steam.

Means is provided for heating the retort to the temperature required for the volatilization of such volatiles as may be contained in the material processed and here shown as gas burners 31, which, when used externally are preferably spaced along the under side of the retort, each individually controllable so that the heat may be varied from one end of the retort to the other as the processing of the material may indicate as desirable.

In the processing of sulphur ore for the extraction of sulphur, the sulphur ore is preferably introduced into the retort in finely divided condition by being manually or mechanically introduced into the hopper 18 and by the worm inducted into the retort. It is well known that sulphur volatilizes approximately at 832° F. The maintenance of the retort at such a temperature would release the larger portion of the sulphur, but it is found desirable to run the retort at a higher temperature to drive off all of the sulphur, for which reason it is found in practice desirable to maintain the temperature of the retort at approximately 950° F.

The length of time during which the sulphur ore shall be processed to extract the entire sulphur content will vary with the ore. Experience seems to indicate that the percentage of sulphur content determines the length of time required and practice will indicate the time required for each particular specimen of ore processed. The time will, however, approximate 45 minutes and such time may be tentatively indicated as the required time, it being understood, however, that this is not a fixed time and that the time will vary as conditions make necessary.

At the opposite end superheated steam is introduced through the pipes 29 and 30 at approximately the retort temperature and is driven by the force of the steam longitudinally through such retort, passing outwardly through the opening 16, carrying therewith the sulphur vapors. The sulphur ore in the meantime is being cascaded through this current of superheated steam by being lifted by the flanges 15 in the retort, thus subjecting it not only to the temperature of the retort but to the action of the superheated steam thereon.

It has been found that a fairly satisfactory extraction of the sulphur may be accomplished without the employment of the superheated steam by merely maintaining the retort at the temperature indicated and continually agitating and cascading the sulphur, but the sulphur is not recovered in as pure condition as when subjected to superheated steam, nor is it liberated as

quickly or readily or as completely. While the invention includes the extraction of sulphur in a retort closed wholly against the introduction of air and subjected to a sufficient temperature, it is not the preferred process, which preferred process is the use of the superheated steam.

It is understood, of course, that the sulphur vapors introduced into the condenser 21 will be condensed and discharged. It is well known that sulphur condenses at approximately 239° F. and it is necessary, therefore, to maintain the condenser at such temperature as will successfully condense the sulphur. The condenser shown is not intended to be a limitation upon the present invention but only to indicate a condenser chamber for the purpose.

What I claim is:

1. The process of extracting sulphur from its ores consisting in charging the sulphur-bearing material into one end of an elongated retort, cascading the material progressively to the opposite end to discharge, introducing a fluid heated to sulphur-vaporizing temperature at the end opposite the charging end and causing a continuous flow of said fluid throughout the length of said retort and the cascading material to liberate and take up the sulphur vapors, taking off the vapor laden fluid at the charging end and condensing the vapors.

2. The process of extracting sulphur from its ores consisting in charging the sulphur-bearing material into one end of an elongated retort, cascading the material progressively to the opposite end to discharge, introducing a fluid heated to sulphur-vaporizing temperature at the end opposite the charging end and causing a continuous flow of said fluid throughout the length of said retort and the cascading material to liberate and take up the sulphur vapors, taking off the vapor laden fluid at the charging end and condensing the vapors, the while maintaining the retort against access of air.

3. The process of extracting sulphur from its ores consisting in charging the sulphur-bearing material into one end of an elongated retort, cascading the material progressively to the opposite end to discharge, introducing steam heated to sulphur-vaporizing temperature at the end opposite the charging end and causing a continuous flow of said steam throughout the length of said retort and the cascading material to liberate and take up the sulphur vapors, taking off the vapor laden steam at the charging end and condensing the vapors.

4. The process of extracting sulphur from its ores consisting in charging the sulphur-bearing material into one end of an elongated retort, cascading the material progressively to the opposite end to discharge, introducing steam heated to sulphur-vaporizing

ing temperature at the end opposite the charging end and causing a continuous flow of said steam throughout the length of said retort and the cascading material to liberate 5 and take up the sulphur vapors, taking off the vapor laden steam at the charging end and condensing the vapors, the while maintaining the retort against access of air.

5. The process of extracting sulphur from 10 its ores consisting in transferring the ores progressively through an elongated retort from a charging end to the opposite end for discharging the spent residuum the while producing a continual redistribution of the 15 mass, introducing steam at a temperature markedly above the vaporization point of sulphur to come in contact with and act first upon the spent material and to travel in opposition to the progression of the sulphur-carrying material and progressively give up 20 its heat in liberating and taking up sulphur vapors, discharging the same at the end opposite its introduction laden with vaporized sulphur and condensing the vapors.
- 25 6. The process of extracting sulphur from its ores consisting in transferring the ores progressively through an elongated retort from a charging end to the opposite end for discharging the spent residuum the while 30 producing continual redistribution of the

mass, introducing steam at a temperature markedly above the vaporization point of sulphur to come in contact with and act first upon the spent material and to travel in opposition to the progression of the sulphur-carrying material and progressively give up 35 its heat in liberating and taking up sulphur vapors, discharging the same at the end opposite its introduction laden with vaporized sulphur and condensing the vapors, the while 40 maintaining the retort against access of air.

7. The process of extracting sulphur from 45 its ores consisting in continuously charging sulphur-carrying material into one end and continuously discharging the residuum from the opposite end of a retort while excluding air therefrom, the while producing continual redistribution of the mass, introducing steam into the discharge end heated to a temperature above the vaporization point of sulphur, 50 said steam traversing the retort to the charging end the while coming in contact with the constantly redistributed surface of said mass, liberating and taking up sulphur vapors en route, discharging the sulphur-laden 55 steam and condensing the vapors.

In testimony whereof I hereunto affix my signature.

EDWARD E. HEDGES.